

UNITED STATES PATENT OFFICE

2,671,021

## POLYMERIC MAGENTA COLOR FORMER

**Sarah C. Kleiger and Henry J. Hugos, Binghamton, N. Y., assignors to General Aniline & Film Corporation, New York, N. Y., a corporation of Delaware**

**No Drawing. Application December 27, 1950,  
Serial No. 203,025**

**18 Claims. (Cl. 95—6)**

1

This invention relates to the production of photographic dye images by color development and particularly to polymeric pyrazolones as color-forming couplers therefor.

Modern methods of color photography utilize multilayer materials having differently sensitized superimposed silver halide emulsion layers, each containing color-forming components fast to diffusion which, upon development with a primary aromatic amino developing agent, yield subtractively colored dyestuff images.

The magenta components most frequently employed are pyrazolone derivatives which are rendered fast to diffusion by the inclusion of a suitable group which imparts a substantive character to the molecule of the component, or of a long chain aliphatic hydrocarbon radical which prevents diffusion of the component in the emulsion. Dye images produced by such components are not entirely satisfactory. The principal disadvantage of these components is their generally waxy character which renders their purification extremely difficult, thus leading to a loss in speed and contrast, undesired color shifts, and stain. The removal of the impurities which cause these undesirable photographic effects is very time-consuming, expensive and not always very effective.

It has also been proposed to react pyrazolones with aliphatic aldehydes to yield dimeric or polymeric color formers. These too, suffer from the above shortcomings and have the added disadvantage of not being interchangeably compatible with gelatin emulsions and other colloidal dispersions, such as modified polyvinyl alcohol which may be used in place of gelatin as a colloidal carrier.

It is an object of the present invention to provide a class of polymeric pyrazolone color formers for producing magenta dye images.

Another object is to provide photographic emulsions containing polymeric pyrazolone color formers capable of yielding, upon color development, dye images of excellent color, high brilliance, stability, and very fine grain.

A further object is to provide photographic emulsions containing polymeric pyrazolones which do not affect the sensitivity of photographic emulsions and do not cause stain.

Other objects and advantages of this invention will be apparent from the following specifications in which its preferred details and embodiments are described.

The above and other objects are accomplished by the use of linear polymers obtained by condensing a dihalide of a dioic acid with a 1-substituted-3-aminopyrazolone to yield a bis-3-aminopyrazolone which is subsequently reacted with an aldehyde.

The linear polymers are compounds whose molecules are chains built up of repeating or recurring units and are characterized by the following general formulae:



wherein R is an alkyl group, e. g., methyl, ethyl, propyl, isopropyl, butyl, isobutyl, amyl, isoamyl, hexyl, heptyl, octyl, an aryl group, e. g., phenyl, tolyl, methoxyphenyl, phenoxyphenyl, chlorophenyl, nitrophenyl, naphthyl, an aralkyl group, e. g., benzyl, methylbenzyl, ethylbenzyl, phenethyl, or a heterocyclic nucleus, e. g., thiazolyl, benzothiazolyl, quinolyl, pyridyl and the like. R<sub>1</sub> is hydrogen or an alkyl, e. g., methyl, ethyl, propyl, butyl, isobutyl, amyl, hexyl, heptyl, octyl, carboxyalkyl, e. g., carboxymethyl, carboxyethyl, carboxypropyl, carboxybutyl, carboxyamyl, cycloalkyl, e. g., cyclopentyl, cyclohexyl, aryl, e. g., phenyl, tolyl, methoxyphenyl, ethoxyphenyl, dimethoxyphenyl, naphthyl, carboxyaryl, e. g., carboxyphenyl, carboxytolyl, carboxynaphthyl, sulfoaryl, e. g., sulphenyl, sulfotolyl, sulfonaphthyl, aralkyl, e. g., benzyl, phenethyl and heterocyclic radicals, e. g., pyridyl, quinolyl, nicotenyl, piperidyl, and wherein —OC—A—CO— is a diacyl radical of a dicarboxylic acid of not more than 18 carbon atoms and selected from the class consisting of aliphatic, cycloaliphatic, aromatic, aromatic-aliphatic, and heterocyclic dicarboxylic acids, e. g., oxalic, malonic, succinic, glutaric, adipic, pimelic, suberic, azelaic, sebacic, heneucanedioic, dodecanedioic, brassylc, tetradeucanedioic, pentadecanedioic, thapsic, fumaric, glutaconic,  $\alpha$ -hydromuconic,  $\beta$ -hydromuconic, 2-ocenedioic, phthalic, isophthalic, terephthalic, 2-methyl-1,4-benzenedicarboxylic, 2-methoxy-1,4-benzenedicarboxylic, 4,4'-dicarboxybibenyl, 1,4-naphthalenedicarboxylic, 3-carboxynaphthylacetyl, 3-carboxynaphthylacetyl, carboxyacrylic, carboxycyclohexaneacetic, camphoric, 1,4-cyclohexanedicarboxylic, pyrazolone dicarboxylic acid, pyridinedicarboxylic and the like, which may be further substituted, for example, by alkyl, alkoxy and halogen, and X represents the number of repeated units in the polymer and is an integer greater than 2.

Examples of polymeric pyrazolones embraced

by the above formulae are the following:

(1)



Polymer of *N,N'*-bis-3-[1-phenyl-5-pyrazolono]urea with formaldehyde

(2)



Polymer of *N,N'*-bis-3-[1-(3'-tolyl)-5-pyrazolono]urea with formaldehyde

(3)



Polymer of *N,N'*-bis-3-[1-(4'-phenoxyphenyl)-5-pyrazolono]urea with formaldehyde

(4)



Polymer of *N,N'*-bis-3-[1-(4'-[p-tert-butyl]phenoxyphenyl)-5-pyrazolono]urea with formaldehyde

(5)



Polymer of *N,N'*-bis-3-[1-(2'-benzothiazolyl)-5-pyrazolono]urea with formaldehyde

(6)



Polymer of *N,N'*-bis-3-[1-(4'-nitrophenyl)-5-pyrazolono]urea with formaldehyde

(7)



Polymer of *N,N'*-bis-3-[1-(3'-tolyl)-5-pyrazolono]oxalyl amide with formaldehyde

(8)



Polymer of *N,N'*-bis-3-[1-(2'-benzothiazolyl)-5-pyrazolono]malonamide with formaldehyde

(9)



Polymer of *N,N'*-bis-3-[1-(4'-phenoxyphenyl)-5-pyrazolono]malonamide with benzaldehyde-2-sulfonic acid



Polymer of *N,N'*-bis-3-[1-ethyl-5-pyrazolono]pimelamide with formaldehydePolymer of *N,N'*-bis-3-[1-phenyl-5-pyrazolono]suberamide with formaldehydePolymer of *N,N'*-bis-3-[1-(4'-methoxyphenyl)-5-pyrazolono]azelaamide with formaldehydePolymer of *N,N'*-bis-3-[1-(4'-bromophenyl)-5-pyrazolono]sebacamide with formaldehydePolymer of *N,N'*-bis-3-[1-(4'-phenoxyphenyl)-5-pyrazolono]sebacamide with p-hydroxybenzaldehydePolymer of *N,N'*-bis-3-[1-phenyl-5-pyrazolono]sebacamide with benzaldehyde-2-sulfonic acid

Polymer of  $N,N'$ -bis-3-[1-(3'-tolyl)-5-pyrazolono]-sebacamide with phthalaldehydic acidPolymer of  $N,N'$ -bis-3-[1-(β-naphthyl)-5-pyrazolono]-dodecanediamide with propionaldehydePolymer of  $N,N'$ -bis-3-[1-phenyl-5-pyrazolono]brassylamide with benzaldehyde-4-sulfonic acidPolymer of  $N,N'$ -bis-3-[1-benzyl-5-pyrazolono]thapsamide with terephthalaldehydic acidPolymer of  $N,N'$ -3-[1-phenyl-5-pyrazolono]terephthalamide with formaldehydePolymer of  $N,N'$ -bis-3-[1-(4'-nitrophenyl)-5-pyrazolono]-isophthalamide with formaldehyde

11

12

(28)

Polymer of *N,N'*-bis-3-[1-phenyl-5-pyrazolono]1,4-cyclohexanediamide with phthalaldehydic acid

(29)

Polymer of *N,N'*-bis-3-[1-phenyl-5-pyrazolono]m-carboxy-cinnamic diamide with formaldehyde

(30)

Polymer of *N,N'*-bis-3-[1-(p-phenoxyphenyl)-5-pyrazolono]-naphthalene-1',4'-dicarboxamide with formaldehyde

(31)

Polymer of *N,N'*-bis-3-[1-phenyl-5-pyrazolono]fumaramide with formaldehyde

(32)

Polymer of *N,N'*-bis-3-[1-phenyl-5-pyrazolono]- $\alpha$ , $\beta$ -diethylsuccinamide with formaldehyde



Brassylyl chloride  
 Tetradecanedioyl chloride  
 Pentadecanedioyl chloride  
 Thapsyl chloride  
 Fumaryl chloride  
 Glutaconyl chloride  
 2-hexenedioyl chloride  
 3-hexenedioyl chloride  
 2-octenedioyl chloride  
 4-amyl-2,5-heptadienedioyl chloride  
 2,9-dimethyl-2,4,6,8-decatetraenedioyl chloride  
 Hexadecanedioyl chloride  
 Phthaloyl chloride  
 Isophthaloyl chloride  
 Terephthaloyl chloride  
 2-methyl-1,4-benzenedicarboxyl chloride  
 2-methoxy-1,4-benzenedicarboxyl chloride  
 1,4-naphthalenedicarboxyl chloride  
 3-carboxylicinnamoyl dichloride  
 3-carboxyldihydrocinnamoyl dichloride  
 3-carboxylphenylacetyl dichloride  
 3-carboxylnaphthylacetyl dichloride  
 4,4'-dicarboxyldiphenyl chloride  
 1,4-cyclohexanedicarboxyl chloride  
 Camphoryl chloride  
 (2-carboxyl-2-methylcyclohexane)acetyl dichloride  
 4,5-pyrazoledicarboxyl chloride  
 3,5-pyridinedicarboxyl chloride

The following compounds are illustrative examples of suitable 3-amino-5-pyrazolones:

3-amino-1-phenyl-5-pyrazolone  
 3-amino-1-(3'-methylphenyl)-5-pyrazolone  
 3-amino-1-(4'-methoxyphenyl)-5-pyrazolone  
 3-amino-1-(4'-phenoxyphenyl)-5-pyrazolone  
 3-amino-1-[4'-(p-tert.-butylphenoxy)phenyl]-5-pyrazolone  
 3-amino-1-[4'-(m-tolyl)phenyl]-5-pyrazolone  
 3-amino-1-[4'-(3',5'-dimethylphenoxy)phenyl]-5-pyrazolone  
 3-amino-1-[3'-chlorophenyl]-5-pyrazolone  
 3-amino-1-(4'-nitrophenyl)-5-pyrazolone  
 3-amino-1-(2'-benzothiazolyl)-5-pyrazolone  
 3-amino-1-(1'-naphthyl)-5-pyrazolone  
 3-amino-1-(2'-naphthyl)-5-pyrazolone  
 3-amino-1-benzyl-5-pyrazolone  
 3-amino-1-phenethyl-5-pyrazolone  
 3-amino-1-(2'-pyridyl)-5-pyrazolone  
 3-amino-1-(2'-quinolyl)-5-pyrazolone

The following are illustrative examples of suitable aldehydes which may be utilized in the polymerization with the bis-amidopyrazolones:

Formaldehyde  
 Acetaldehyde  
 Propionaldehyde  
 Butyraldehyde  
 Iso-butyraldehyde  
 Valeraldehyde  
 Iso-Valeraldehyde  
 Caproaldehyde  
 Glyoxylic acid  
 Formylacetic acid  
 $\beta$ -Formylpropionic acid  
 Formylsuccinic acid  
 $\epsilon$ -Formylcaproic acid  
 Cyclopentanecarboxaldehyde  
 Benzaldehyde  
 1-naphthaldehyde  
 o-Tolualdehyde  
 m-Tolualdehyde  
 p-Tolualdehyde

4-methoxybenzaldehyde  
 3-methoxybenzaldehyde  
 2-methoxybenzaldehyde  
 4-ethoxybenzaldehyde  
 5 3-ethoxybenzaldehyde  
 2-ethoxybenzaldehyde  
 Benzaldehyde-4-sulfonic acid  
 Benzaldehyde-2-sulfonic acid  
 3,4-dimethoxybenzaldehyde  
 10 Phthalaldehydic acid  
 Isophthalaldehydic acid  
 Terephthalaldehydic acid  
 Nicotinaldehyde  
 Cinchoninaldehyde  
 15 3-quinolinecarboxaldehyde  
 1-piperidine carboxaldehyde  
 2-pyridylpropionaldehyde  
 Phenylacetaldehyde  
 Phenylpropionaldehyde

20 The polymeric pyrazolones prepared in accordance with the present invention are added to the silver halide emulsion in the form of a solution or a suspension in a suitable solvent such as an aqueous, alcoholic or aqueous-alcoholic one normal solution of sodium or potassium hydroxide. Dispersing agents such as isopropylnaphthalene sulfonic acid or other suitable dispersing agents, for example, those disclosed in United States Patent 2,186,717, may be used in preparing the suspensions of the polymeric pyrazolones for incorporation into silver halide emulsions. Instead of gelatin, the polymeric pyrazolones may be incorporated into other colloidal materials such as water dispersible organic esters of cellulose, polyamides, hydroxyethyl cellulose, or modified polyvinyl alcohol. The polymeric pyrazolones have the unique property of being compatible not only with gelatinous silver halide emulsions but also with those which contain a synthetic colloidal carrier as a substitute for gelatin.

As examples of suitable aromatic primary amino developing agents which may be employed for the development of the color forming polymers of the present invention, there may be mentioned 4-aminoaniline, 4-ethylaminoaniline, 2-diethylaminoaniline, 4-dialkylaminoanilines, e.g., 4-dimethylaminoaniline, 4-diethylaminoaniline, 4-[N-( $\beta$ -hydroxyethyl)-N-ethyl]aminoaniline, 4-( $\beta$ , $\beta$ -dihydroxyethyl)aminoaniline, 4-amino-N-ethyl-N-( $\beta$ -methanesulfonamidoethyl)-2-methylaniline sulfate and the like. These developing agents are preferably used in the form of their salts, such as the hydrochloride, since they are more soluble and stable than the free base. They are characterized by the presence of a free or primary amino group in the aromatic nucleus which enables the oxidation product of the developer to couple with the polymeric color former to form a dye image of the azomethine type in the emulsion. The silver image which is developed simultaneously may be removed by bleaching and fixing in the well known manner to leave the color image in the emulsion.

A suitable developing solution can be prepared as follows:

|                                     | Grams |
|-------------------------------------|-------|
| 4-diethylaminoaniline hydrochloride | 2     |
| 70 Sodium carbonate (anhydrous)     | 50    |
| Sodium sulfite (anhydrous)          | 2     |
| Potassium bromide                   | 0.2   |
| Water to make 1 liter.              |       |

The exposed silver halide emulsions containing the polymeric color-formers are developed in the

17

above solution in the usual manner. A black and white first developer and a second exposure are only employed if the desired image is to be of the reversal type.

The invention is further illustrated by the following examples, but it is to be understood that the invention is not to be restricted thereto.

18

absorption maximum at 535 m $\mu$ . and did not show any indications of diffusibility. The magenta image was characterized by the fineness of its grain, and showed greater than average stability on storage at elevated temperatures and high humidity as well as increased resistance to acid fumes.

### *Example II*



## Polymer of N,N'-bis-3-[1-phenyl-5-pyrazolono]adipamide with formaldehyde

### *Example I*



## Polymer of N,N'-bis-3-[1-phenyl-5-pyrazolono]urea with formaldehyde

8.75 grams (0.05 mole) of 1-phenyl-3-amino-5-pyrazolone and 25 mls. of pyridine were mixed and warmed on a steam bath. 7.3 grams of a 35% solution of phosgene in benzene (containing 2.56 grams or 0.025 mole of phosgene) were added dropwise to the mixture. Heating and stirring were continued for an additional 45 minutes. The reaction mixture was cooled to room temperature. A white product separated which was filtered off, washed with pyridine and dried in vacuo at room temperature using concentrated sulfuric acid as a desiccant. The product can be further purified by recrystallization from hot pyridine. The product decomposes when heated above 260° C.

20 42.5 grams (0.24 mole) of 1-phenyl-3-amino-5-pyrazolone and 120 mls. of pyridine were heated together on a steam bath. To this mixture, 23 grams (0.125 mole) of adipyl chloride were added dropwise with stirring. After 2 hours of continued stirring and heating, the mixture was poured into 300 mls. of water. The precipitated bis-amidopyrazolone was filtered and first washed with water and then with dilute ammonia. The residue was dried and melted at 281-4° C.

36 A mixture consisting of 11.5 grams (0.025 mole) of the dried bis-amidopyrazolone, 125 mls. of dioxane, 2 mls. of a 37% formalin (0.025 mole) and 50 drops of pyridine was heated under reflux on a steam bath for 4 hours. An additional 35 0.4 ml. of formalin was added in order to provide a slight excess of formalin and the refluxing continued for 1 hour. An insoluble product was filtered from the hot mixture and washed with 40 dioxane. 10 grams of the product decomposing above 270° C. were obtained.

A bright and intense magenta dye image having a maximum absorption at  $530 \text{ m}\mu$  was produced by utilizing the above color former as in Example I. The dye image was characterized by the fineness of its grain.

### Example III



### Polymer of $N,N'$ -bis-3-[1-(3'-tolyl)-5-pyrazolono]adipamide with benzaldehyde-2-sulfonic acid

1.87 grams (0.005 mole) of the above bis-amidopyrazolone, 25 mls. of dioxane, 0.4 ml. of a 37% solution of formalin (0.005 mole) and ten drops of pyridine were mixed and refluxed for two hours. In order to provide a slight excess of formaldehyde, 0.1 ml. of formalin was added at this point and the heating continued for an additional 3 hours. The mixture was filtered while hot and the residue washed with dioxane. The yield of the dried material was 1.79 grams.

0.35 gram of the above color former was dispersed in a small volume of dilute aqueous alkali and the dispersion added to 50 mls. of a gelatinous silver halide emulsion. The emulsion was coated onto a suitable support and dried. The dried film was sensitometrically exposed and developed in a 4-diethylaminoaniline developer. The brilliant magenta image obtained had an

46 grams (0.24 mole) of 1-(3'-tolyl)-3-amino-5-pyrazolone and 120 mls. of pyridine were heated together on a steam bath. To this mixture, 23 grams (0.125 mole) of adipyl chloride were added dropwise with stirring. After 2 hours of continued stirring and heating, the mixture was poured into 300 mls. of water. The precipitated bis-amidopyrazolone was filtered, and first washed with water and then with dilute ammonia, and subsequently dried.

A mixture of 11.9 grams (0.027 mole) of the dried bis-amidopyrazolone and 250 mls. of di-oxane was heated on a steam bath. To this mixture, 5 grams (0.028 mole) of the sodium salt of benzaldehyde-2-sulfonic acid and 50 drops of pyridine were added and the mixture was heated for 4 hours on the steam bath under reflux. The mixture was filtered while hot and the filtrate

19

poured into approximately 1 liter of cold water. The resultant solution was acidified by the addition of hydrochloric acid until a polymerization product separated as a fine, tan-colored precipitate.

The final product can be further purified by washing with hot ethanol. A bright and dense magenta image was obtained by utilizing the color former as in Example I. The dye image was characterized by the fineness of its grain.

20

77 grams (0.44 mole) of 1-phenyl-3-amino-5-pyrazolone were mixed with 220 mls. of pyridine and warmed on a steam bath with stirring. 53 grams (0.22 mole) of sebacyl chloride were added dropwise with stirring. Heating and stirring were continued for 3 hours. After cooling, the mixture was poured into 500 mls. of cold water while stirring. The precipitated product was purified by stirring with dilute ammonia, washed with water and dried. Further purification can be ob-

*Example IV*



Polymer of *N,N'*-bis-3-[1-phenyl-5-pyrazolone]terephthalamide with formaldehyde

17.5 grams (0.1 mole) of 1-phenyl-3-amino pyrazolone were dissolved in 60 mls. of hot pyridine and the solution heated to reflux. 10.3 grams (0.05 mole) of terephthalyl chloride dissolved in 50 mls. of dioxane were added gradually to the boiling mixture. After the addition had been completed, refluxing was continued for another hour. The larger portion of the solvents present was then distilled off and the hot residue poured into water. A tarry product separated which became granular upon acidification with hydrochloric acid. The precipitate was filtered off, washed with water and dried in a vacuo over concentrated sulfuric acid. The final product can be further purified by boiling out with hot ethanol.

25 obtained by consecutive washings with alcohol and ether. The product melted at 251-3°C.

2.1 grams (0.004 mole) of the bis-amidopyrazolone were dispersed in 25 mls. of dioxane, treated with 0.4 ml. of 37% of formalin (0.15 gram or 0.005 mole of formaldehyde) and 10 drops 30 of pyridine. The mixture was heated under reflux on a steam bath for 5 hours. The solution was filtered hot and poured into 100 mls. of water. The finely divided product was made more readily filterable by the addition of hydrochloric acid.

35 A magenta dye image of good density and brilliance was obtained when the above color former was utilized in the silver halide emulsion as in Example I. The dye image obtained was characterized by the fineness of its grain.

*Example VI*



Polymer of *N,N'*-bis-3-[1-phenyl-5-pyrazolone]sebacamide with benzaldehyde-2-sulfonic acid

2.4 grams (0.005 mole) of the above bis-amidopyrazolone and 25 mls. of dioxane were mixed with 0.4 ml. formalin (containing 0.15 gram or 0.005 mole of formaldehyde) and 10 drops of pyridine. The mixture was heated for 4 hours on a steam bath under reflux. The dioxane-insoluble fraction was filtered off and purified by washing with dioxane. A bright and dense magenta dye image was produced by utilizing the above color former as in Example I. The dye image was characterized by the fineness of its grain.

55 1 gram (0.0019 mole) of the bis-amidopyrazolone of Example V was mixed with 0.4 gram (0.0019 mole) of the sodium salt of benzaldehyde-2-sulfonic acid in 25 mls. of dioxane. The suspension was refluxed for 3 hours to yield a clear light brown solution. The solution was filtered and the filtrate diluted with 100 mls. of water to give a milky suspension which was acidified with hydrochloric acid, whereupon the polymer separated in a filterable form.

60 A bright and dense magenta image was ob-

*Example V*



Polymer of *N,N'*-bis-3-[1-phenyl-5-pyrazolone]sebacamide with formaldehyde

tained when this polymeric color former was incorporated in a gelatin silver halide emulsion as in Example I. It was particularly characterized by the fineness of the developed color grains.

*Example VII*



Polymer of *N,N'*-bis-3-[1-phenyl-5-pyrazolone]sebacamide with p-hydroxybenzaldehyde

Example VI was repeated with the exception that 0.24 gram of p-hydroxybenzaldehyde was used in place of 0.4 gram (0.0019 mole) of the sodium salt of benzaldehyde-2-sulfonic acid. When a dispersion of this color former was added to a silver halide emulsion, a magenta image of above average density and fineness of grain was obtained after color development.

*Example VIII*



Polymer of *N,N'*-bis-3-[1-phenyl-5-pyrazolone]sebacamide with phthalaldehydic acid

2.1 grams (0.005 mole) of the sebacylamide-bis-pyrazolone of Example VI, 25 mls. of dioxane, 10 drops of pyridine and 0.75 gram (0.005 mole) of phthalaldehydic acid were refluxed for 5 hours to yield a dark brown solution. The solution was filtered while hot and the filtrate poured into 100 mls. of water. The finely divided precipitate was aggregated by the addition of strong hydrochloric acid. The precipitate was filtered, washed with water, and dried in vacuo to give a light colored product.

A bright and dense magenta image was produced by utilizing the above color former as in Example I. The dye was characterized by the fineness of its grain.

Various modifications of the invention will occur to persons skilled in this art and we, therefore, do not intend to be limited in the patent granted except as by the appended claims.

We claim:

1. A photographic silver halide emulsion containing a polymeric coupler compound of the class consisting of compounds having the following formulae:



and



wherein R represents a member selected from the class consisting of alkyl, aryl, aralkyl and heterocyclic groups, R<sub>1</sub> represents a member selected from the class consisting of hydrogen,

alkyl, aryl, aralkyl and heterocyclic radicals, -OC-A-CO- represents a radical of a di-carboxylic acid of not more than 18 carbon atoms and is selected from the class consisting of aliphatic, cycloaliphatic, aromatic, aliphatic-aromatic, and heterocyclic dicarboxylic acids, and X represents the number of repeated units in the polymer and is an integer greater than 2.

2. A photographic silver halide emulsion containing as a color former, the polymer of *N,N'*-bis-3-[1-phenyl-5-pyrazolone]urea with formaldehyde.

3. A photographic silver halide emulsion containing as a color former, the polymer of *N,N'*-bis-3-[1-(3'-tolyl)-5-pyrazolone]adipamide with benzaldehyde-2-sulfonic acid.

4. A photographic silver halide emulsion containing as a color former, the polymer of *N,N'*-bis-3-[1-phenyl-5-pyrazolone]terephthalamide with formaldehyde.

5. A photographic silver halide emulsion containing as a color former, the polymer of *N,N'*-bis-3-[1-phenyl-5-pyrazolone]sebacamide with formaldehyde.

6. A photographic silver halide emulsion containing as a color former, the polymer of *N,N'*-bis-3-[1-phenyl-5-pyrazolone]sebacamide with phthalaldehydic acid.

7. The method of producing a magenta photographic image in a silver halide emulsion layer which comprises exposing the layer and developing it with a solution of an aromatic primary amino developing agent, said emulsion layer containing as a magenta color former, a polymeric coupler compound of the class consisting of compounds having the following general formulae:



and



and



wherein R represents a member selected from the class consisting of alkyl, aryl, aralkyl, and heterocyclic groups, R<sub>1</sub> represents a member selected from the class consisting of hydrogen, alkyl, cycloalkyl, aryl, aralkyl, and heterocyclic radicals, —OC—A—CO— represents a radical of a dicarboxylic acid of not more than 18 carbon atoms and is selected from the class consisting of aliphatic, cycloaliphatic, aromatic, aliphatic-aromatic and heterocyclic dicarboxylic acids, and X represents the number of repeated units in the polymer and is an integer greater than 2.

8. The method of producing a magenta photographic image in a silver halide emulsion layer which comprises exposing and developing it with a solution of an aromatic primary amino developing agent, said emulsion containing as a magenta color former, the polymer of N,N'-bis-3-[1-phenyl-5-pyrazolono]urea with formaldehyde.

9. The method of producing a magenta photographic image in a silver halide emulsion layer which comprises exposing and developing it with a solution of an aromatic primary amino developing agent, said emulsion containing as a magenta color former, the polymer of N,N'-bis-3-[1-(3'-tolyl)-5-pyrazolono]adipamide with benzaldehyde-2-sulfonic acid.

10. The method of producing a magenta photographic image in a silver halide emulsion layer which comprises exposing and developing it with a solution of an aromatic primary amino developing agent, said emulsion containing as a magenta color former, the polymer of N,N'-bis-3-[1-phenyl-5-pyrazolono]terephthalamide and formaldehyde.

11. The method of producing a magenta photographic image in a silver halide emulsion layer which comprises exposing and developing it with a solution of an aromatic primary amino developing agent, said emulsion containing as a magenta color former, the polymer of N,N'-bis-3-[1-phenyl-5-pyrazolono]sebacamide with formaldehyde.

12. The method of producing a magenta photographic image in a silver halide emulsion layer which comprises exposing and developing it with a solution of an aromatic primary amino developing agent, said emulsion containing as a magenta color former, the polymer of N,N'-bis-3-[1-phenyl-5-pyrazolono]sebacamide with phthalaldehydic acid.

13. A photographic element comprising a support and a silver halide emulsion layer, said emulsion layer containing as a color former for the magenta image, a polymeric coupler compound of the class consisting of compounds having the following formulae:



wherein R represents a member selected from the class consisting of alkyl, aryl, aralkyl, and heterocyclic groups, R<sub>1</sub> represents a member selected from the class consisting of hydrogen, alkyl, carboxyalkyl, cycloalkyl, aryl, sulfoaryl, carboxyaryl, aralkyl, and heterocyclic radicals, and wherein —OC—A—CO— represents a radical of a dicarboxylic acid of not more than 18 carbon atoms and selected from the class consisting of aliphatic, cycloaliphatic, aromatic, and heterocyclic dicarboxylic acids, and X represents the number of repeated units in the polymer and is an integer greater than 2.

14. A photographic element comprising a support and a silver halide emulsion layer, said emulsion layer containing as a color former for the magenta image, the polymer of N,N'-bis-3-[1-phenyl-5-pyrazolono]urea with formaldehyde.

15. A photographic element comprising a support and a silver halide emulsion layer, said emulsion layer containing as a color former for the magenta image, the polymer of N,N'-bis-3-[1-(3'-tolyl)-5-pyrazolono]adipamide with benzaldehyde-2-sulfonic acid.

16. A photographic element comprising a support and a silver halide emulsion layer, said emulsion layer containing as a color former for the magenta image, the polymer of N,N'-bis-3-[1-phenyl-5-pyrazolono]terephthalamide with formaldehyde.

17. A photographic element comprising a support and a silver halide emulsion layer, said emulsion layer containing as a color former for the magenta image, the polymer of N,N'-bis-3-[1-phenyl-5-pyrazolono]sebacamide with formaldehyde.

18. A photographic element comprising a support and a silver halide emulsion layer, said emulsion layer containing as a color former for the magenta image, the polymer of N,N'-bis-3-[1-phenyl-5-pyrazolono]sebacamide with phthalaldehydic acid.

SARAH C. KLEIGER.  
HENRY J. HUGOS.

## References Cited in the file of this patent

## UNITED STATES PATENTS

| Number    | Name               | Date          |
|-----------|--------------------|---------------|
| 2,186,734 | Schneider          | Jan. 9, 1940  |
| 2,186,849 | Wilmanns et al.    | Jan. 9, 1940  |
| 2,380,032 | Dorough et al.     | July 10, 1945 |
| 2,511,231 | Weissberger et al. | June 13, 1950 |

## FOREIGN PATENTS

| Number  | Country       | Date          |
|---------|---------------|---------------|
| 562,675 | Great Britain | July 12, 1944 |